

## UNITED STATES PATENT OFFICE

2,449,980

## REMOVAL OF PHOTOGRAPHICALLY ACTIVE INGREDIENTS FROM GELATIN

Rudolph E. Damschroder and Marie E. Kauffman, Rochester, N. Y., assignors to Eastman Kodak Company, Rochester, N. Y., a corporation of New Jersey.

No Drawing. Application September 14, 1946,  
Serial No. 697,156

7 Claims. (Cl. 260—118)

1

This invention relates to the removal of photographically active ingredients from gelatin or other proteins by treating the gelatin or other proteins with certain metals in finely divided form.

Photographic emulsions are ordinarily prepared by incorporating a photo-sensitive silver salt in gelatin in aqueous solution as the protective coating for the photo-sensitive silver salt. As gelatin is a material which is obtained from natural sources, there is oftentimes considerable variation in the properties of that material when used photographically. For instance, some types of gelatin have therein a considerable proportion of photographically active ingredients. Because of this variation, it has heretofore been difficult to prepare photographic emulsion of uniform properties following a set formula for their preparation.

One object of our invention is to provide a method for treating gelatin or other proteins whereby a considerable proportion of the photographically active ingredients thereof are removed or rendered inactive. Another object of our invention is to provide a method for treating gelatin or other proteins with metals in finely divided condition. Other objects of our invention will appear herein.

We have found that the photographically active ingredients of gelatin or other proteins are either removed or rendered inactive by treating the gelatin or other proteins with active metals whose sulfides are insoluble and which will not adversely affect the photographic emulsion which is formed therefrom. Our process in its broadest aspects comprises treating the protein either in aqueous or non-aqueous solution in liquid form with one of the metals under the designation given, in finely divided condition and thereafter subjecting the solution to filtration to remove the metal particles therefrom. As it is desirable that the gelatin be in liquid form, ordinarily the operation will be carried out at a temperature within the range of 30-75° C. Ordinarily, the most convenient procedure is to dissolve the protein in an inert solvent and contact the metal particles therewith. Where the protein is water-soluble as in the case of gelatin, albumin, etc., the use of an aqueous dissolving liquid is desirable. If desired, however, non-aqueous solvents may be used; for instance, gelatin may be dissolved in formamide and treated with the finely divided metal.

Gelatins and other proteins vary among themselves as to the degree of photographic activity

which is present therein. Accordingly, some proteins will need to be treated for a longer time and with a greater amount of metal per unit weight of protein than will other proteins having less photographic activity. However, even with the gelatins or other proteins having a high degree of photographic activity, the use of metal in an amount which will not render the photographically active ingredients entirely inactive will at least reduce the photographic activity of the gelatin, if only a partial reduction in activity is desired. Unless, however, only partial reduction in activity is desired, it is ordinarily desirable to use a large excess of metal so that every portion of the gelatin or other protein is contacted with the metal particles.

Our invention is adapted to the treatment of various types of gelatin. For instance, hydrolyzed gelatins may be treated in accordance with our invention to inactivate photographically active materials therein as well as gelatins which have not been subjected to hydrolysis and which have not been subjected to any degrading treatment. We have found that the treatment in accordance with our invention works equally well on gelatin made from different raw stocks, such as green, salted calfskin, acidulated bone, or dried hide stock. Our invention is also adapted to the treatment of proteins generally, if desirable, to inactivate the photographically active materials which are present therein. For instance, casein, zein, albumen, soy bean protein or the like may be treated with a finely divided metal in accordance with our invention.

We have also found that the process works very well within quite a reasonable range of pH. For instance, gelatins with pH values within the range of 4 to 9 have been deactivated in accordance with our process, and there has been but little variation in the results obtained. We have found that there is no necessity for adjusting the pH to any particular value in the carrying out of our process. If the metal which is employed is susceptible to the action of acid, it is preferable to treat therewith only those proteins having a pH of above 6.

The metals which are employed to treat gelatin in accordance with our invention should be in a condition in which a large amount of surface is exposed which is ordinarily in a finely divided condition. If the process is operated by incorporating the finely divided metal into the gelatin solution, it is ordinarily desirable to obtain the best results that the particle size of the metal be

at least 150-mesh or smaller although in some cases a larger particle size may be desirable.

The materials which are suitable for use in our process are those, the sulfides of which, are insoluble in water and which will not adversely affect a photographic emulsion. The metals which are not suitable are those the sulfides of which are soluble in water or which hydrolyze rapidly in water solution or which have a derogatory effect upon photographic emulsions. Some of the metals which in finely divided form are adapted for use in our process are platinum, nickel, cobalt, cadmium, and silver. One of the finely divided metals which we have found to be particularly suitable in processes in accordance with our invention is Raney nickel which is a well-recognized catalytic material. Another finely divided material which is useful is Adams catalyst, which is finely divided platinum prepared by reducing platinum oxide, also a well-known catalytic material.

The following examples illustrate our invention:

*Example 1.*—1½ g. of Raney nickel were stirred into a 12% aqueous gelatin solution made up using 1 pound of dry gelatin. The stirring was continued for ½-¾ hour at 40° C. The solid materials were then removed from the gelatin by filtering through a Kiefer press. The resulting solution was chilled, dried down, and was found to be useful for photographic emulsions, and the photographically active ingredients of that gelatin had been rendered inactive or removed as indicated by the loss in developed silver density of the emulsion made with the treated gelatin as compared to that of the untreated gelatin.

*Example 2.*—The procedure of Example 1 was repeated with each of the following metals in finely divided form: cobalt, platinum, lead and ordinary nickel. The gelatin which was obtained in each case was found to be useful for photographic emulsions and the photographically active ingredients thereof had been inactivated.

It appears that in the process in accordance with our invention there is a chemical combination which takes place between the metal particles and the photographically active materials, and after the treatment of the protein, the metal particles and any reaction product formed therefrom are removed from the mass.

We claim:

1. A method of treating a protein having inherent photographically active ingredients therein to render those photographically active ingredients inactive which comprises treating the protein while in solution with a finely divided metal selected from the group consisting of platinum,

nickel, cobalt, lead, cadmium, and silver, followed by removing the metal particles and any reaction products thereof from the protein.

2. A method of treating gelatin having inherent photographically active ingredients therein to render those photographically active ingredients inactive which comprises treating the gelatin while in solution with a finely divided metal selected from the group consisting of platinum, nickel, cobalt, lead, cadmium, and silver, followed by removing the metal particles and any reaction products thereof from the protein solution.

3. A method of treating gelatin having inherent photographically active ingredients therein to render those photographically active ingredients inactive which comprises treating an aqueous solution of the gelatin with a finely divided metal selected from the group consisting of platinum, nickel, cobalt, lead, cadmium, and silver, followed by removing the metal particles and any reaction products thereof from the gelatin solution.

4. A method of treating gelatin having inherent photographically active ingredients therein to render those ingredients inactive which comprises treating a solution of gelatin having a pH within the range of 4-9 with a finely divided metal selected from the group consisting of platinum, nickel, cobalt, lead, cadmium, and silver, followed by removing the metal particles and any reaction products thereof from the gelatin.

5. A method of treating gelatin having inherent photographically active ingredients therein to render those ingredients inactive, which comprises treating an aqueous solution of the gelatin with finely divided Raney nickel, followed by removing the Raney nickel and any reaction products thereof from the gelatin by filtering.

6. A method of treating gelatin having inherent photographically active ingredients therein to render those ingredients inactive, which comprises treating an aqueous solution of the gelatin with finely divided platinum, followed by removing the platinum and any reaction products thereof from the gelatin solution by filtering.

7. A method of treating gelatin having inherent photographically active ingredients therein to render those ingredients inactive, which comprises dissolving the gelatin in water, treating the gelatin for a time with finely divided Raney nickel, and then separating the Raney nickel and any reaction products thereof from the gelatin.

RUDOLPH E. DAMSCHRODER.  
MARIE E. KAUFFMAN.